

# UNITED STATES PATENT OFFICE.

FOSTER MILLIKEN, OF LAWRENCE, NEW YORK, ASSIGNOR TO FOSTER MILLIKEN,  
S. FULLERTON WEAVER, AND JAMES M. REPLIER, AS TRUSTEES.

## ALLOY.

1,354,988.

Specification of Letters Patent.

Patented Oct. 5, 1920.

No Drawing.

Application filed October 8, 1919. Serial No. 329,186.

To all whom it may concern:

Be it known that I, FOSTER MILLIKEN, a citizen of the United States, and a resident of Lawrence, in the county of Nassau, and 5 State of New York, have invented a new and Improved Alloy, of which the following is a full, clear, and exact description.

The object of the invention is to provide a new and improved alloy especially designed as a special acid resisting metal at 10 high temperatures and also as a high temperature metal.

The alloy contains the following metals in substantially the following proportions, 15 namely:

|        |          |           |
|--------|----------|-----------|
| Copper | 50 to 60 | per cent. |
| Nickel | 28 to 36 | " "       |
| Zinc   | 4 to 8   | " "       |
| Iron   | 4 to 8   | " "       |

20

These metals are melted together and the resultant alloy is very efficacious as an acid resisting metal used particularly for resisting the principal acids, alkalis, and mixtures, also to resist high temperatures. 25

This alloy differs from the one described in the Letters Patent of the United States, No. 1,310,363, granted to me on July 15, 1919, by the low percentages of the zinc and iron and the increased percentage of nickel. 30

I claim:

An alloy consisting of the following ingredients in substantially the following proportions, namely:

|        |          |           |
|--------|----------|-----------|
| Copper | 50 to 60 | per cent. |
| Nickel | 28 to 36 | " "       |
| Zinc   | 4 to 8   | " "       |
| Iron   | 4 to 8   | " "       |

35

FOSTER MILLIKEN.